

# UNITED STATES PATENT OFFICE.

LLOYD R. RHOADES, OF FREMONT, OHIO, ASSIGNOR, BY MESNE ASSIGNMENTS, TO  
NATIONAL CARBON COMPANY, INC., A CORPORATION OF NEW YORK.

## ELECTRIC BATTERY.

1,273,000.

Specification of Letters Patent.

Patented July 16, 1918.

No Drawing.

Application filed January 5, 1916. Serial No. 70,407.

*To all whom it may concern:*

Be it known that I, LLOYD R. RHOADES, a citizen of the United States, residing at Fremont, in the county of Sandusky and State of Ohio, have invented a certain new and useful Improvement in Electric Batteries, of which the following is a full, clear, and exact description.

My invention relates to electric batteries, and more particularly to bibulous linings for so-called dry cells.

As is well known, a dry cell consists of a zinc can with a paper or other bibulous lining inside of which is compacted a battery mix around a central electrode. It has been the practice to apply a paste of flour and water or other analogous materials to the bibulous lining before the mix is tamped in the cell. Sometimes this paste has been smeared on the linings by hand and sometimes by applying it with a paint brush.

I have found that much better results are obtained in dry cells if the flour paste is applied as a uniform coating by spraying the paste on the linings. The sprayed coating is preferably dried on the lining before the latter is placed in the zinc can. In this way a very uniform coat is obtained and the paste seems to be slightly forced into the pores of the lining which makes it adhere to the lining much better than when the paste is brushed or smeared on.

When a uniform coating is applied to the lining by spraying, as above described, the local action is reduced and the electrolytic action during service is uniform throughout the surface of the zinc. When the flour paste is painted on the lining with a brush for ex-

ample, the coating is not uniform and the corrosion of the zinc seems to depend upon the thickness of the paste, so that the bristle marks are plainly discernible on a zinc electrode after the cell has been placed on the shelf for a long enough time to show corrosion.

I am not sure of the reason for the reduced corrosion in dry cells with sprayed coating, and it may be that it is due to concentration effects. That is, the concentration in the thick portion of the paste might be different from that in the thin portion, and a difference of voltage would be set up due to such difference in concentration. This would tend to cause corrosion on open circuit, as well as on closed circuit. However, regardless of any theory, it has been demonstrated to be a fact that the sprayed coating produces superior results.

The paste can be sprayed on the lining with any spraying device, such as the usual paint sprayer. The paste used may also be of any desired nature, such as pastes of flour either raw or cooked, meal, cornstarch, etc.

Having described my invention, what I claim is:—

1. A dry cell containing a bibulous lining having a uniform coating of flour and water paste adherent thereto.
2. A dry cell having a lining with a coating of flour and water paste uniformly applied to the same and forced into the surface pores.

In testimony whereof, I hereunto affix my signature.

LLOYD R. RHOADES.